

86

Nov. 8, 1938.

J. A. BABOR

2,135,554

METHOD OF MANUFACTURING FORMED OR MOLDED ARTICLES

Filed March 9, 1937

Fig. 1.



Fig. 2.



INVENTOR

Joseph A. Babor.

Gustav R. Thompson,

ATTORNEY

XR

## UNITED STATES PATENT OFFICE

2,135,554

METHOD OF MANUFACTURING FORMED OR  
MOLDED ARTICLES

Joseph A. Babor, New York, N. Y.

Application March 9, 1937, Serial No. 129,782

4 Claims. (Cl. 18—48)

This invention relates to the manufacture of formed or molded articles (pipe coverings, blocks, boards and the like) from exfoliated zonolite and the like and provides an improved method for such manufacture with improved properties in the product.

The invention provides an improved method of manufacturing formed or molded articles from exfoliated zonolite (vermiculite) and the like and a binder, by which the mixing and handling of the material is greatly facilitated, the fracturing of the zonolite during the mixing process minimized, the cost of manufacturing reduced, and a lighter and less heat conducting article obtained. The heat insulating properties of the formed or molded product are enhanced.

An embodiment of apparatus for use in carrying out the process, is illustrated in the accompanying drawing, wherein:

20 Fig. 1 is a vertical longitudinal sectional view of said embodiment; and

Fig. 2 is a detailed view in side elevation of a part of a belt used in conjunction with the hopper for feeding material to molds.

25 According to the present invention I take a discrete mass of exfoliated zonolite which has the properties of taking up or absorbing a liquid or liquid solvent, and the particles of which have a diminishable volume, mix it with a binder in a dry finely divided state, and thereafter soften the binder, or give it adhesive properties, with a solvent or liquid to unite the exfoliated zonolite particles or the like in the form or shape of the article desired. The solvent or liquid 30 which is used to soften the binder mixed with the zonolite is advantageously introduced into the mixture in an absorbed state, that is the solvent is absorbed in the zonolite or the like prior to the mixing of the zonolite with the dry binder, 35 and the mixing thereafter with dry binder is carried on so as to not expel the absorbed solvent. At the end of the mixing operation the batch has substantially the appearance and discreteness of the original mass of flaky material, 40 and is apparently dry.

45 The mixture, with the solvent absorbed in the zonolite, is put into molds, or other apparatus for forming or shaping the same, and the exfoliated zonolite is compressed to an extent that 50 solvent or liquid is squeezed or forced out so as to wet and soften the binder so that the exfoliated zonolite particles will be united and stuck together, and the discrete mass united in the form or shape of article desired. The mass is held under compression for such a time as neces-

sary for the binding material to assume the active properties of a binder. This may be a matter of moments or of a few minutes, depending upon the nature of the binding material and the liquid or solvent used. Thereafter the mass may be dried to remove (and to recover if this is profitable) the solvent or liquid used for softening or transforming the binder. After drying, the molded or shaped articles is ready for storage or use. A few hours to a day, depending on the binder used, is sufficient for the binder to "set". The drying may be hastened by the use of an oven or dryer. The mixture may also be applied and formed in the manner of a plaster, that is by the use of a trowel or hawk or similar instrument by which the mass may be compressed and shaped.

55 The amount of liquid or solvent which is added to the exfoliated zonolite is such as to substantially saturate and be absorbed by the exfoliated zonolite. The liquid or solvent may be added to the exfoliated zonolite in any suitable way, and if an excess of the liquid or solvent over that which the exfoliated zonolite will hold by absorption is used, the excess is drained or otherwise removed, prior to the addition of the dry binder.

10 The dry binder may be any one or more suitable for the purpose in view and the solvent or liquid used is that which is appropriate to dissolving or otherwise uniting with the dry binder used to transform it to an active binding material.

15 Examples of suitable binders (in dry form) and of a solvent or liquid appropriate therefor are enumerated as follows:

|                         |                                                                                            |
|-------------------------|--------------------------------------------------------------------------------------------|
| Cement                  | water.                                                                                     |
| Glue                    | water acidulated or<br>not with acetic acid.                                               |
| Shellac                 | alcohol.                                                                                   |
| Casein glue             | water.                                                                                     |
| Magnesium chloride      | water containing alkalis of sufficient concentration to produce a basic salt of magnesium. |
| Magnesium sulfate       | water containing alkalis of sufficient concentration to produce a basic salt of magnesium. |
| Bakelite (soluble form) | acetone and special mixtures.                                                              |
| Glyptol resin           | acetone and special mixtures.                                                              |

86 2

2,135,554

In the drawing there is illustrated an apparatus in which the process may be carried out for forming heat insulating pipe coverings.

Referring to said drawing, numeral 10 designates a mixer of a type to mix discrete material without substantial compression. As here shown, the mixer 10 comprises a vessel 11 having a central rotatable shaft 12 therein provided with blades 13. The shaft 12 is arranged to be rotated very slowly in a direction to turn the blades to exert a lifting action on the material within the vessel, so as to cause a circulation which is upward at the center and downward at the sides. The discrete material, zonolite and the like, is placed in the mixer 10. As heretofore described the solvent or liquid for softening the binder is contained in the zonolite or the like, in the absorbed state. To this end, the liquid or solvent may be introduced into the mixer through a spout 15 for example, before the binder is added to the mixture. The zonolite or the like could, however, be introduced into the mixer 10 with the liquid or solvent already absorbed therein.

Sufficient liquid or solvent could be added to the zonolite to immerse the same, and the excess of that which the zonolite is capable of holding by absorption removed by draining, or in other suitable manner. The same thing could be accomplished, by running into the mixer 10 such an amount of the solvent or liquid which will be absorbed by the zonolite.

When the liquid or solvent has been added in the manner described, the zonolite remains in a discrete form with the liquid or solvent which has been added thereto within the inner interstices of the zonolite.

Binding material, in the dry state, and preferably finely divided, is then added to the material in the mixer 10, and thorough mixing effected in such manner as not to compress the material and thereby expel the liquid or solvent contained therein. The mixture retains the properties of a dry mass.

After the mixing in the mixer 10 is completed, the mixture is advantageously dumped into a hopper 18. The hopper 18 may be located near a table 20 for supporting a mold 22 in a position to receive batches of the mixture from the hopper 18. After the mold 22 is filled, it may be transferred to a means for compressing the material therein, here shown in the form of a cam actuated tamper 25. The tamper acts to compress the exfoliated zonolite, or similar material, and expel from the interstices therein some of the liquid or solvent contained or absorbed therein. The expelled liquid or solvent wets the binder and causes it to acquire active properties as a binder, so that it will unite and bind the particles of the zonolite or like material. Binders such as cement are hydrated and made soft or plastic, and set by crystallization. Binders such as glue and the like dissolve, soften, and harden when dry. The compression is maintained long enough to enable the binder to soften or hydrate. Compression maintained for a few moments, in the case of cement and water, will be sufficient. In the case of shellac and alcohol, compression maintained up to 10 minutes may be required.

After the binder is softened, or become plastic, so as to adhere to the zonolite or the like, the pressure may be relieved from the molded article. The mold and the molded material therein may be removed for air drying, or transferred

to a dryer. The dryer, where the liquid or solvent is worth recovering, may be of a type for recovering the solvent.

After the material has been acted on by the tamper 25, and before removal to a dryer or the like, it may be transferred to a means for shaping the face of the material in the mold, which shaping means may be a cam actuated shaper 27. The compression and shaping may however, be done together, in which case the two functions may be performed by the device 27.

For transferring the mold 22 from the filling position to the tamper 25 (or to the tamper 25 and shaper 27) a conveyor, as an intermittently operated belt conveyor 30, may be provided.

The hopper 18 at its lower end is provided with means 35, for feeding batches of the material to successive molds 22. The feeding means 35 is advantageously in the form of a belt 37 having fins 38 pivotally mounted thereon as indicated at 39. Abutments 40 are provided for supporting the fins in one direction against turning. The space between adjacent fins forms a pocket 41, into which the material in the hopper 18 falls.

The material in the pocket 41 is so light that it does not readily fall out of the pocket at the dumping position, especially if the material in the pockets has been pressed to the extent of squeezing some of the liquid or solvent out of the particles which come in contact with the fins, and thereby causes adhesion. To facilitate the dumping of material from the pockets 41 at the dumping position, the fins are provided with arms 44, and a cam 45 is provided for co-acting with the arms 44 to turn the fins 38 at the dumping position, in a direction to enlarge the pocket and thereby facilitate the falling therefrom of the material in the pocket.

A water or air jet 50 is preferably provided for removing any material or adhesive remaining on the fins after the material has been dumped from the pockets, and before the fins again enter the hopper.

The mold 22 in the filling position, is filled with the mixture (carrying the absorbed liquid or solvent) to a heaping amount. The quantity of the material or mixture in the mold has an excess of the order of 10 to 15 percent of the flush capacity of the mold.

Articles formed or molded from exfoliated vermiculite or zonolite according to the present process are exceptionally light and porous, and have exceptionally good heat insulating properties.

The present process particularly facilitates the handling of exceptionally light weight material, which, at some stage of the manufacturing process, must be mixed with an adhesive binder. When exceptionally light weight material such as exfoliated material is mixed with an adhesive binder it is not easily manipulatable in apparatus, because gravity has but small effect thereon, and masses of the material stick to surfaces when many other materials admixed with adhesives would readily fall from such surfaces.

The process effects economies in manufacture, and the finished product has improved properties by reason of the fact that the interstices within the mass of the zonolite are less filled with the binder than when made according to previously used methods.

The process may be carried out by other modes

of procedure than that herein specifically described.

What is claimed is:

1. A method of making molded or formed articles (pipe coverings, blocks, boards and the like) from compressible exfoliated zonolite or the like, and a binder, comprising adding to the exfoliated zonolite a liquid in an amount to substantially saturate and be absorbed within the exfoliations 5 of the zonolite said liquid being of a kind which acts with the binder to make it active as a binder, adding a binder in a dry finely divided state to the zonolite containing the absorbed liquid mixing, and, after mixing, expelling liquid from 10 within the exfoliations of the zonolite to soften the binder to unite the zonolite particles in the form or shape of article desired.

2. A method of making molded or formed articles (pipe coverings, blocks, boards and the like), from compressible exfoliated zonolite or the like, and a binder, comprising adding to the exfoliated zonolite a liquid in an amount to substantially saturate and be absorbed within the exfoliations of the zonolite, said liquid being of 15 a kind which acts with the binder to make it active as a binder, adding a binder in a dry finely divided state to the zonolite containing the absorbed liquid, mixing, and, after mixing, compressing the mixture to expel liquid from within 20 the exfoliation of the zonolite to soften the binder to unite the zonolite particles in the form or shape of article desired.

3. A method of making molded or formed articles (pipe coverings, blocks, boards and the like) 25 from compressible exfoliated zonolite or the like, and a binder, comprising adding to the exfoliat-

ed zonolite a liquid in an amount to substantially saturate and be absorbed within the exfoliations of the zonolite, said liquid being of a kind which acts with the binder to make it active as a binder, adding a binder in a dry finely divided state to the zonolite containing the absorbed liquid, mixing, and, after mixing, compressing the mixture to expel liquid from within 5 the exfoliations of the zonolite to soften the binder to unite the zonolite particles in the form or shape of article desired, and maintaining the pressure on the mixture for a few seconds to a few minutes until the binder takes up the requisite amount of the liquid to enable it to act effectively to bind the zonolite particles. 10

4. A method of making molded or formed articles (pipe coverings, blocks, boards and the like), from compressible exfoliated zonolite or the like, and a binder, comprising adding to the exfoliated zonolite a liquid in an amount to substantially saturate and be absorbed within the capillaries of the zonolite, said liquid being of a kind which acts with the binder to make it active as a binder, adding a binder in a dry finely divided state to the zonolite containing the absorbed liquid, mixing, and, after mixing, compressing the mixture to expel liquid from within 15 the exfoliations of the zonolite to soften the binder to unite the exfoliated zonolite particles in the form or shape of article desired, and maintaining the pressure on the mixture for a few seconds to a few minutes until the binder takes up the requisite amount of the liquid to enable it to act effectively to bind the zonolite particles, and drying to remove liquid. 20

JOSEPH A. BABOR.